

1,406,498.

Patented Feb. 14, 1922.

J. A. RYMER.  
PROCESS FOR ENAMELING WOOD OR METAL SURFACES.  
APPLICATION FILED JULY 15, 1919.



Inventor.

John A. Rymer.  
By A.S. Paré  
Attorney.

# UNITED STATES PATENT OFFICE.

JOHN A. RYMER, OF OAKLAND, CALIFORNIA, ASSIGNOR OF ONE-HALF TO EDWARD V. TIFFANY, OF OAKLAND, CALIFORNIA.

## PROCESS FOR ENAMELING WOOD OR METAL SURFACES.

1,406,498.

Specification of Letters Patent. Patented Feb. 14, 1922.

Application filed July 15, 1919. Serial No. 311,063.

To all whom it may concern:

Be it known that I, JOHN A. RYMER, a citizen of the United States, and a resident of Oakland, county of Alameda, State of California, have invented certain new and useful Improvements in Processes for Enameling Wood or Metal Surfaces, whereof the following is a specification.

This invention relates to a process for 10 enameling wood or metal surfaces.

The accompanying drawing forming part 15 of the specification illustrates the body and the coatings of materials, the same bearing legends to indicate what they represent.

15 In carrying out the invention I proceed as follows, viz:—If the surface is an old one, that is, one that has been painted or varnished before, I first remove all old paint from the surface, by any suitable method.

20 I then wash the surface with gasoline or alcohol to kill the effect of the paint or varnish removed. If the surface is metal, I now treat it with a metal primer which has

25 an elastic and adherent quality. When this primer is thoroughly dry, if the surface is rough, I build it up with a putty made of lacquer and dry white lead, and when it is thoroughly smoothed, I coat it with japan color of the color which it is to finally have.

30 This coating I repeat as often as necessary to produce a solid color. I then apply an intermediate or protection coat, which is to be made of straight japan, or japan and litharge (a half pound to the gallon) and japan color the same as before. This coating

35 is best sprayed on, and all parts should be thoroughly covered. I then proceed as follows: I then take of celluloid enamel, or similar enamel, one-third enamel, one-third lacquer and one-third slow drying thinner.

40 I spray the entire surface with this mixture, and when dry rub it to a dead smooth finish, and repeat the treatment till the desired 45 gloss and finish is acquired. The surface may then be rubbed with pumice stone and water.

The same process is applied to wood surfaces, except that instead of the metal 50 primer, a primer made of white lead, linseed oil and japan is used.

After each spraying when the coating has dried and hardened, the surface is treated by rubbing with pumice stone and water.

Having thus described my process in full, 55 clear and exact terms required by law, and knowing that it comprises novel, useful and valuable improvements in the art to which it pertains, I here state that I do not wish to be limited to the precise terms, steps and 60 arrangements of the several parts, as herein set forth, as the same may be variously modified without departing from the spirit thereof.

It is to be understood that certain terms 65 employed in this specification are those which designate certain well known articles of commerce in the painters' supply trade.

The term "metal primer" refers to a composition in which linseed oil, red lead and 70 turpentine are ingredients. The term "lacquer" used herein is understood to be a composition, the base of which is celluloid treated with amyl acetate or acetone. The term "japan color" refers to a coating, comprising 75 a pigment such as drop black, parisian blue or the like, ground in nonpareil japan. "Slow drying thinner" is composed of acetone and castor oil in approximately the proportions of one-half ounce of castor oil 80 to a gallon of acetone.

What I claim and desire to secure by Letters Patent of the United States, is the following, to wit:—

1. The process of treating surfaces which 85 consists in priming the surface, then treating it with japan color one or more times, then giving it an intermediate coat containing japan, and then treating it one or more 90 times with a mixture containing one-third celluloid enamel, one-third lacquer and one-third slow drying thinner, and rubbing after each such treatment.

2. The process of treating surfaces, which 95 consists in priming the surface, smoothing it with lacquer and dry white lead, treating it one or more times with japan color, giving it an intermediate coat containing japan, and treating it one or more times with a mixture 100 containing one-third celluloid enamel, one-third lacquer, and one-third slow drying thinner, and rubbing after each treatment.

3. The process of treating surfaces, which 105 consists in priming the surface and smoothing the same, then coating it one or more times with japan color, then spraying it with an intermediate coat containing japan, then

spraying it one or more times with a mixture containing one-third of celluloid enamel, or similar enamel, one-third lacquer and one-third slow drying thinner, and rubbing, when dry, to a smooth finish with pumice stone and water after each such spraying.

In testimony that I claim the foregoing I have hereto set my hand this 21st day of June, 1919, in the presence of witnesses.

JOHN A. RYMER.

Witnesses:

OLIVE TEXDAHL,  
F. L. WOLFE.